

## UNITED STATES PATENT OFFICE

2,541,521

## TREATMENT OF CAST IRON

Harry B. Kinnear and George P. Krumlauf, Columbus, Ohio, assignors, by mesne assignments, to Chromium Mining & Smelting Corporation, Limited, Sault Ste. Marie, Ontario, Canada, a corporation of Ontario

No Drawing. Application November 14, 1945,  
Serial No. 628,664

12 Claims. (Cl. 75—56)

1

This invention relates to metallurgy and has for an object the provision of certain improvements in metallurgical methods or processes. More particularly, the invention contemplates the provision of certain improvements in methods or processes suitable for use in the production of cast iron. A particular object of the invention is to provide an improved method or process for improving the mechanical or physical properties of cast iron. A specific object of the invention is to provide a method or process for treating cast iron to improve its mechanical or physical properties.

The invention is based on our discovery that cast iron can be treated while in the molten state with a nitrate to produce cast iron products having improved mechanical or physical properties. Thus, for example, we have found that by reacting with a nitrate, molten cast iron, such as cupola iron and blast furnace iron, containing not less than about two and one-half percent (2.5%) of carbon and about one per cent (1.0%) of elemental silicon, cast iron products having improved transverse, tensile, deflection, impact, hardness and other properties can be produced. The method or process of the invention is particularly useful for treating gray cast iron to improve its properties. The use of nitrate for treating cast iron in accordance with the invention has little or no effect on the depth of chill.

In carrying out a method or process of the invention, molten cast iron from any suitable source is reacted in a ladle, for example, with a nitrate in amount sufficient to modify the mechanical or physical properties or characteristics of the cast iron without altering substantially the composition of the cast iron with respect to carbon and silicon. The percentage of carbon in the cast iron may be altered about 0.03 to 0.06 percent, or about 1 to 2 percent of the actual carbon content, and the percentage of silicon in the alloy may be altered about 0.06 to 0.13 percent, or about 4 to 7 percent based on the actual amount of silicon present in the cast iron.

Any suitable nitrate may be employed in carrying out a method of the invention. A single nitrate may be employed in treating a bath of molten cast iron, or the bath of molten cast iron may be treated with two or more nitrates singly or in admixture. Nitrates of sodium, strontium, barium, calcium and copper may be employed with particular advantage in carrying out a method or process of the invention. The nitrates may be employed in any suitable amounts which by reaction with the cast iron will not seriously alter the composition of the cast iron with respect to carbon and silicon. We have employed nitrates in amounts by weight equal to about four-tenths of one percent (0.4%) to about one and one-quarter percent (1.25%) of the weight of the cast iron treated.

2

The following examples illustrate results obtained in carrying out methods or processes of the invention employing various nitrates in the amounts in treating in ladles sixty pound batches of molten cast iron products of the compositions indicated:

| 10                                | Reagent Added                     | Weight of Addition, Lb. | Metal Analyses |             |             |            |
|-----------------------------------|-----------------------------------|-------------------------|----------------|-------------|-------------|------------|
|                                   |                                   |                         | Per Cent T. C. | Per Cent Mn | Per Cent Si | Per Cent N |
| No addition                       |                                   |                         | 3.15           | .54         | 1.50        | .002       |
| NaNO <sub>3</sub>                 | 0.50                              | 3.12                    | .50            | 1.41        | .009        |            |
| Ba(NO <sub>3</sub> ) <sub>2</sub> | 0.50                              | 3.14                    | .52            | 1.44        | .009        |            |
| No addition                       |                                   |                         | 3.25           | .56         | 1.61        | .003       |
| NaNO <sub>3</sub>                 | 0.50                              | 3.21                    | .51            | 1.52        | .008        |            |
| Ba(NO <sub>3</sub> ) <sub>2</sub> | 0.50                              | 3.24                    | .54            | 1.57        | .008        |            |
| Sr(NO <sub>3</sub> ) <sub>2</sub> | 0.50                              | 3.19                    | .52            | 1.51        | .011        |            |
| No addition                       |                                   |                         | 3.15           |             | 1.88        | .002       |
| NaNO <sub>3</sub>                 | 0.25                              | 3.14                    |                | 1.84        |             | .004       |
| Do                                | 0.50                              | 3.12                    |                | 1.80        |             | .005       |
| Do                                | .75                               | 3.12                    |                | 1.75        |             | .005       |
| 20                                | Ca(NO <sub>3</sub> ) <sub>2</sub> | .50                     | 3.09           |             | 1.84        | .008       |
| No addition                       |                                   |                         | 3.29           |             | 1.58        | .004       |
| NaNO <sub>3</sub>                 | .25                               | 3.28                    |                | 1.55        |             | .006       |
| Do                                | .50                               | 3.27                    |                | 1.52        |             | .006       |
| Cu(NO <sub>3</sub> ) <sub>2</sub> | .50                               | 3.27                    |                | 1.56        |             | .006       |
| Ca(NO <sub>3</sub> ) <sub>2</sub> | .50                               | 3.25                    |                | 1.52        |             | .011       |

| 30                                | Reagent Added                     | Weight of Addition, Lb. | Mechanical Properties of Test Bars |                          |                     |
|-----------------------------------|-----------------------------------|-------------------------|------------------------------------|--------------------------|---------------------|
|                                   |                                   |                         | Trans-verse, Lb.                   | Tensile, Lb. per Sq. In. | Deflec-tion, Inches |
| No addition                       |                                   |                         | 2,760                              | 37,450                   | .305                |
| NaNO <sub>3</sub>                 | 0.50                              | 3,180                   | 43,450                             | .297                     |                     |
| Ba(NO <sub>3</sub> ) <sub>2</sub> | 0.50                              | 3,040                   | 42,300                             | .300                     |                     |
| No addition                       |                                   |                         | 2,570                              | 38,250                   | .202                |
| 35                                | NaNO <sub>3</sub>                 | 0.50                    | 3,260                              | 50,075                   | .323                |
| Ba(NO <sub>3</sub> ) <sub>2</sub> | 0.50                              | 3,065                   | 46,650                             | .312                     |                     |
| Sr(NO <sub>3</sub> ) <sub>2</sub> | 0.50                              | 3,155                   | 48,250                             | .297                     |                     |
| No addition                       |                                   |                         | 2,690                              | 36,350                   | .299                |
| NaNO <sub>3</sub>                 | 0.25                              | 3,085                   | 39,450                             | .331                     |                     |
| Do                                | 0.50                              | 3,085                   | 41,150                             | .304                     |                     |
| Do                                | .75                               | 3,185                   | 40,900                             | .340                     |                     |
| 40                                | Ca(NO <sub>3</sub> ) <sub>2</sub> | .50                     | 3,080                              | 38,550                   | .329                |
| No addition                       |                                   |                         | 2,825                              | 37,500                   | .322                |
| NaNO <sub>3</sub>                 | .25                               | 3,048                   | 41,500                             | .322                     |                     |
| Do                                | .50                               | 3,240                   | 43,900                             | .320                     |                     |
| Cu(NO <sub>3</sub> ) <sub>2</sub> | .50                               | 3,125                   | 42,700                             | .312                     |                     |
| Ca(NO <sub>3</sub> ) <sub>2</sub> | .50                               | 3,215                   | 43,350                             | .280                     |                     |

| 50                                | Reagent Added                      | Weight of Addition, Lb. | Impact, Ft.-Lb. | B. H. N. 3,000 kg. Load | Chill, Inches |
|-----------------------------------|------------------------------------|-------------------------|-----------------|-------------------------|---------------|
|                                   |                                    |                         |                 |                         |               |
| No addition                       |                                    |                         | 45.50           | 199                     |               |
| NaNO <sub>3</sub>                 | 0.50                               | 52.00                   | 220             |                         |               |
| Ba(NO <sub>3</sub> ) <sub>2</sub> | 0.50                               | 52.00                   | 216             |                         |               |
| No addition                       |                                    |                         | 43.50           | 199                     |               |
| NaNO <sub>3</sub>                 | 0.50                               | 55.60                   | 228             |                         |               |
| Ba(NO <sub>3</sub> ) <sub>2</sub> | 0.50                               | 52.75                   | 224             |                         |               |
| Sr(NO <sub>3</sub> ) <sub>2</sub> | 0.50                               | 55.00                   | 226             |                         |               |
| No addition                       |                                    |                         | 49.00           | 193                     | 10/16         |
| 55                                | NaNO <sub>3</sub>                  | 0.25                    | 56.00           | 203                     | 8/16          |
| Do                                | 0.50                               | 58.75                   | 205             |                         | 10/16         |
| Do                                | .75                                | 58.50                   | 208             |                         | 9/16          |
| Ca(NO <sub>3</sub> ) <sub>2</sub> | .50                                | 57.25                   | 207             |                         | 10/16         |
| No addition                       |                                    |                         | 51.50           | 198                     | 14/16         |
| NaNO <sub>3</sub>                 | .25                                | 58.00                   | 206             |                         | 16/16         |
| NaNO <sub>3</sub>                 | .50                                | 55.00                   | 209             |                         | 15/16         |
| Cu(NO <sub>3</sub> ) <sub>2</sub> | .50                                | 53.00                   | 212             |                         | 14/16         |
| 60                                | Ca (NO <sub>3</sub> ) <sub>2</sub> | .50                     | 59.00           | 213                     | 17/16         |

We claim:

1. The method of treating cast iron which comprises reacting the cast iron while molten with one or more nitrates in amount by weight equal to about four-tenths of one percent (0.4%) to about one and one-quarter percent (1.25%) of the weight of the cast iron and sufficient to modify the mechanical or physical characteristics or properties of the cast iron.

2. The method of treating cast iron which comprises reacting the cast iron while molten with one or more nitrates including sodium nitrate in amount by weight equal to about four-tenths of one percent (0.4%) to about one and one-quarter percent (1.25%) of the weight of the cast iron and sufficient to modify the mechanical or physical characteristics or properties of the cast iron.

3. The method of treating cast iron which comprises reacting the cast iron while molten with one or more nitrates including strontium nitrate in amount by weight equal to about four-tenths of one percent (0.4%) to about one and one-quarter percent (1.25%) of the weight of the cast iron and sufficient to modify the mechanical or physical characteristics or properties of the cast iron.

4. The method of treating cast iron which comprises reacting the cast iron while molten with one or more nitrates including barium nitrate in amount by weight equal to about four-tenths of one percent (0.4%) to about one and one-quarter percent (1.25%) of the weight of the cast iron and sufficient to modify the mechanical or physical characteristics or properties of the cast iron.

5. The method of treating cast iron containing not less than two and one-half percent of carbon and one percent of elemental silicon which comprises reacting the cast iron while molten with one or more nitrates in amount by weight equal to about four-tenths of one percent (0.4%) to about one and one-quarter percent (1.25%) of the weight of the cast iron and sufficient to modify the mechanical or physical characteristics or properties of the cast iron.

6. The method of treating cast iron containing not less than two and one-half percent of carbon and one percent of elemental silicon which comprises reacting the cast iron while molten with one or more nitrates including sodium nitrate in amount by weight equal to about four-tenths of one percent (0.4%) to about one and one-quarter percent (1.25%) of the weight of the cast iron and sufficient to modify the mechanical or physical characteristics or properties of the cast iron.

7. The method of treating cast iron containing not less than two and one-half percent of carbon and one percent of elemental silicon which comprises reacting the cast iron while molten with one or more nitrates including strontium nitrate in amount by weight equal to about four-tenths of one percent (0.4%) to about one and one-quarter percent (1.25%) of the weight of the cast iron and sufficient to modify the mechanical or physical characteristics or properties of the cast iron.

5 8. The method of treating cast iron containing not less than two and one-half percent of carbon and one percent of elemental silicon which comprises reacting the cast iron while molten with one or more nitrates including barium nitrate in amount by weight equal to about four-tenths of one percent (0.4%) to about one and one-quarter percent (1.25%) of the weight of the cast iron and sufficient to modify the mechanical or physical characteristics or properties of the cast iron.

10 9. The method of treating gray cast iron which comprises reacting the cast iron while molten with one or more nitrates in amount by weight equal to about four-tenths of one percent (0.4%) to about one and one-quarter percent (1.25%) of the weight of the cast iron and sufficient to modify the mechanical or physical characteristics or properties of the cast iron.

15 10. The method of treating gray cast iron which comprises reacting the cast iron while molten with one or more nitrates including sodium nitrate in amount by weight equal to about four-tenths of one percent (0.4%) to about one and one-quarter percent (1.25%) of the weight of the cast iron and sufficient to modify the mechanical or physical characteristics or properties of the cast iron.

20 11. The method of treating gray cast iron which comprises reacting the cast iron while molten with one or more nitrates including strontium nitrate in amount by weight equal to about four-tenths of one percent (0.4%) to about one and one-quarter percent (1.25%) of the weight of the cast iron and sufficient to modify the mechanical or physical characteristics or properties of the cast iron.

25 12. The method of treating gray cast iron which comprises reacting the cast iron while molten with one or more nitrates including barium nitrate in amount by weight equal to about four-tenths of one percent (0.4%) to about one and one-quarter percent (1.25%) of the weight of the cast iron and sufficient to modify the mechanical or physical characteristics or properties of the cast iron.

30 HARRY B. KINNEAR.  
GEORGE P. KRUMLAUF.

#### REFERENCES CITED

The following references are of record in the file of this patent:

#### UNITED STATES PATENTS

| Number    | Name          | Date          |
|-----------|---------------|---------------|
| 412,448   | Archbold      | Oct. 8, 1889  |
| 661,406   | Leiby         | Nov. 6, 1900  |
| 2,174,740 | Graham et al. | Oct. 3, 1939  |
| 2,243,783 | Udy           | May 27, 1941  |
| 2,280,872 | Udy           | Apr. 28, 1942 |
| 2,339,673 | Boegehold     | Jan. 18, 1944 |

#### FOREIGN PATENTS

| Number | Country       | Date    |
|--------|---------------|---------|
| 798    | Great Britain | Of 1866 |